

May 9, 1933.

H. M. NAUGLE ET AL

1,908,171

MAKING BLOOMS, SLABS, AND BILLETS

Filed April 17, 1932

3 Sheets-Sheet 1



May 9, 1933.

H. M. NAUGLE ET AL

1,908,171

MAKING BLOOMS, SLABS, AND BILLETS

Filed April 17, 1932

3 Sheets-Sheet 2



Fig. 4



Fig. 5



Fig. 6



Fig. 7

Inventors

H. M. Naugle  
A. J. Townsend

By  
Grease and Bishop Attorneys

May 9, 1933.

H. M. NAUGLE ET AL

1,908,171

MAKING BLOOMS, SLABS, AND BILLETS

Filed April 17, 1932

3 Sheets-Sheet 3



Fig.9



Fig.8



Fig.10



Fig.11



Fig.12

By

H. M. Naugle  
A. J. Townsend  
Grease and Bishop Attorneys

## UNITED STATES PATENT OFFICE

HARRY M. NAUGLE AND ARTHUR J. TOWNSEND, OF CANTON, OHIO, ASSIGNEES TO  
NAUGLE & TOWNSEND, INC., OF WILMINGTON, DELAWARE, A CORPORATION OF  
DELAWARE

## MAKING BLOOMS, SLABS, AND BILLETS

Application filed April 7, 1932. Serial No. 603,764.

The invention relates to the centrifugal molding, straightening and rolling of steel blooms, slabs, billets and the like; and this application is a continuation in part of the 5 common subject matter of our copending application, Serial No. 448,602, filed April 30, 1930, entitled "Making blooms, slabs and billets".

One of the objects of the present improvements is to make an annular ring by centrifugally molding molten metal to form a ring with such an external shape or configuration that when the ring is severed to form one or more arcuate blooms, and the blooms are 15 given a roll pass through a stand of plain or grooved rolls, straightened blooms, slabs or billets issue from the rolls.

It is a further object of the present invention to make a molded annular ring having a 20 thickness at its inner circumference sufficient- ly greater than the thickness at its outer circumference, that the inner peripheral area of the ring is substantially the same as the outer peripheral area thereof.

Another object of the present invention is to centrifugally mold an annular ring, sever 25 the ring to form one or more arcuate blooms, and then straighten the arcuate blooms, by pressure rolling and compressing the metal 30 between rolls engaging the upper and lower surfaces of the blooms as distinguished from the arcuate surfaces thereof.

A further object of the present invention is to centrifugally mold an annular ring, 35 sever the ring to form one or more arcuate blooms having opposite arcuate surfaces and opposite non-parallel surfaces, then straighten the arcuate blooms by rolling the same to compress the blooms between the opposite 40 non-parallel surfaces, and then reduce the straightened blooms to form billets or slabs.

The centrifugal molding of the annular rings may be carried out by utilizing the method of making blooms, slabs and billets 45 disclosed in our copending application, Serial No. 465,303, filed July 2, 1930, and the rate of cooling and solidification of different portions or regions of the ring may be controlled by applying a blanket of heat insulat- 50 ing material to the inner face of the ring, as

disclosed in our copending application, Serial No. 563,583, filed September 18, 1931.

Some types of heat insulating materials utilized for forming a heat insulating blanket on the inner arcuate face of a centrifugally 55 molded ring may adhere to the inner face of the ring and to the corresponding arcuate surface of an arcuate bloom severed therefrom; and it may not in certain cases be desirable to perform a major cleaning opera- 60 tion to remove the heat insulating material from the arcuate face of the arcuate bloom.

It is therefore a further object of the present invention to straighten an arcuate bloom having opposite arcuate surfaces and oppo- 65 site non-parallel surfaces, which may have insulating material adhering to one of its arcuate surfaces, by pressure rolling the arcuate bloom to apply pressure to the non-par- 70 allel surfaces so as to displace the metal at and adjacent to the said arcuate surface, so that any heat insulating material, which may be adhering thereto cracks or drops away from the bloom, or is loosened so that it is subsequently very easily removed therefrom 75 by a simple or minor cleaning operation.

The inner annular or arcuate surface of a centrifugally molded ring may sometimes be slightly concaved from the upper to the lower surfaces thereof, and the upper and lower in- 80 ner annular corners of the ring may some- times be sharp. Preparatory to carrying out roll reducing operations, it is desirable, if not necessary, to eliminate the concavity in the arcuate face of arcuate blooms severed from 85 such rings and to eliminate sharp corners from the blooms.

It is therefore a further object of the pres- 90 ent invention to straighten an arcuate bloom having opposite arcuate surfaces and oppo- site non-parallel surfaces, in which one of the arcuate surfaces may be slightly concaved be- 95 tween the opposite non-parallel surfaces and in which the corners between said arcuate surface and the non-parallel surfaces may be sharp, by pressure rolling the arcuate blooms to apply pressure to the non-parallel surfaces and displace or extrude the metal in the bloom at and adjacent to its depressed arcu- 100 ate surface and sharp corners for eliminating

the depression or concavity and sharp corners.

And finally, it is an object of the present invention to provide a simplified, inexpensive and convenient method of making blooms, slabs, billets and the like, which eliminates many usual steps or operations carried out in prevailing practice.

These and other objects may be obtained by carrying out the improved method disclosed herein and illustrated diagrammatically in the accompanying drawings forming part hereof, in which

Figure 1 is a sectional view of a centrifugally molded annular ring made and utilized in carrying out the improved method;

Fig. 2 is a diagrammatic plan view of a roller table and hot saw for severing the ring shown in Fig. 1 to form one or more arcuate blooms, a conveyor, a furnace charging device, a holding furnace, and a stand of grooved rolls, which may be utilized for carrying out the improved method;

Fig. 3 is a perspective view of an arcuate bloom severed from the ring shown in Fig. 1;

Fig. 4 is an enlarged fragmentary elevation of a three high stand of grooved rolls, which may be utilized for straightening and then reducing the arcuate bloom shown in Fig. 3;

Fig. 5 is an enlarged section through the arcuate bloom shown in Fig. 3;

Fig. 6 is an enlarged section through the bloom after it has been given a straightening pass on the rolls shown in Fig. 4;

Fig. 7 is a perspective view of a billet which may be produced from the straightened bloom by reducing the same by a plurality of passes on the rolls shown in Fig. 3;

Fig. 8 is a perspective view of an arcuate slab which may be utilized for rolling plates;

Fig. 9 is an enlarged fragmentary elevation of a three high stand of plain rolls, which may be utilized for straightening and/or reducing the arcuate slab shown in Fig. 8;

Fig. 10 is an enlarged section through the arcuate slab shown in Fig. 8;

Fig. 11 is an enlarged section through the slab after it has been given a straightening pass on the rolls shown in Fig. 9; and

Fig. 12 is a perspective view of a plate, which may be produced from the straightened slab by reducing the same by a plurality of passes on the rolls shown in Fig. 9.

Similar numerals refer to similar parts throughout the drawings.

In carrying out the improved method, the preferably continuous annular ring 20 is centrifugally molded by introducing fluid molten metal at a temperature of 2600° F. and upwards into a rapidly rotating annular mold, wherein the molten metal by the action of centrifugal force assumes a ring shape. Immediately thereafter, a blanket or coating of heat insulating material is preferably de-

posited on the inner face of the rotating ring to control the cooling of different regions of the ring.

After the centrifugal molding of the ring has been completed, the same is removed from the mold and transferred to the roller table 21 for being severed by the hot saw 22 to form one or more arcuate blooms 23. The ring 20 is molded to have a generally trapezoidal shape in cross section with opposite upper and lower non-parallel surfaces 24 and 25, respectively, and opposite outer and inner arcuate surfaces 26 and 27 respectively, and with rounded corners 28 between the upper and lower surfaces 25 and outer arcuate surface 26.

The inner arcuate surface 27 of the ring 20 may sometimes be slightly concaved as shown at 29 between the upper and lower surfaces 24 and 25, and may also have sharp corners 30 between the inner concaved arcuate surface 27—29 and the upper and lower surfaces 24 and 25.

When certain types of heat insulating materials are utilized for forming a heat insulating blanket on the inner arcuate face of a centrifugally molded ring, the blanket of the same may adhere to the inner face of the ring after it has been removed from the centrifugal molding machine and severed, as indicated diagrammatically at 31 in Figs. 1 and 3.

The arcuate blooms 23 are conveyed by a conveyor 32 from the roller table 21 to the charging end of the holding furnace 34, where a furnace charging device 35 may be utilized for charging them into the furnace 34. The arcuate blooms 23 are heated to the desired rolling temperature in the holding furnace 34, after which they are removed as indicated at 23a and are passed through the rolls generally indicated at 36 in Fig. 2 wherein the arcuate blooms 23 are straightened to form the straight bloom diagrammatically indicated by dot-dash lines at 23b in Fig. 2.

In passing the arcuate blooms through the rolls 36, the upper and lower non-parallel surfaces 24 and 25 are engaged by the rolls to compress the blooms between the opposite non-parallel surfaces and thereby straighten the blooms as they issue from the rolls. When it is desired to roll billets from the blooms, the mill 36 may comprise grooved rolls shown more or less diagrammatically in Fig. 4 in which the straightening pass is indicated generally at 37. A cross section through the arcuate bloom is shown in Fig. 5 immediately before the bloom is passed through the straightening pass 37, while Fig. 6 shows a cross section of the straightened bloom after it issues from the straightening pass 37.

The roll pass 37 is designed so that the upper and lower surfaces 24 and 25 of the bloom are not only compressed by the pressure ap-

plied thereto by the rolls, but they are also depressed as indicated diagrammatically at 24a and 25a in Fig. 6, so that the concaved arcuate surface 27-29 of the arcuate bloom 5 is displaced and extruded outward to remove the concavity during the straightening pass as indicated diagrammatically at 29a in Fig. 6.

The displacement of the metal at and adjacent 10 the concaved surface 29 likewise loosens or cracks away any insulating material which may have adhered to that surface, so as to avoid the necessity of performing a major cleaning operation to remove the heat insulating material; and the straightening roll 15 pass 37 also removes the sharp corners 30 so that the straightened bloom 23b shown in Fig. 6 has rounded corners 28a.

The straightened bloom 23b may then be 20 given a desired number of passes through the grooved rolls shown in Fig. 4 to produce billets 38 of any desired size, such as shown in Fig. 7.

When it is desired to roll plates, the ring 25 may be molded so that arcuate slabs such as shown at 40 in Fig. 8 may be severed from the ring, which may be straightened and rolled on the mill 36 which may comprise plain rolls shown at 41 in Fig. 9. A cross 30 section through the arcuate slab 40 is shown in Fig. 10 immediately before the slab is given a straightening pass through the rolls 41, while Fig. 11 shows a cross section of the 35 straightened slab 40a after it issues from the straightening pass.

The arcuate slab 40 not only has its upper and lower non-parallel surfaces engaged by and compressed by the pressure applied thereto by the rolls 41, but the arcuate surface 40' thereof, which may be very slightly concaved, is displaced and extruded to remove the concavity during the straightening pass, as indicated diagrammatically at 40a' in Fig. 11.

The displacement of the metal at and adjacent to the concave surface 40' likewise loosens or cracks away any insulating material which may have adhered to that surface following the centrifugal molding operation.

The straightened bloom 40a may then be given a desired number of passes through the rolls 41 to produce plates 42 of any desired size, such as shown in Fig. 12.

The rings 20, having cross sections for being severed to produce either the arcuate blooms 23 or the arcuate slabs 40, preferably have a cross sectional area of some sixteen square inches and a circumferential length of some twenty-five feet. However, when it is desired to produce larger blooms, slabs, billets and the like, the rings 20 may be molded to have larger cross sectional areas and/or circumferential lengths.

In carrying out the improved method, 65 which includes centrifugally molding an an-

nular ring having a generally trapezoidal cross section, severing the ring to form one or more arcuate blooms, then compressing and roll straightening the arcuate blooms by applying pressure to the non-parallel surfaces thereof, and then reducing the straightened blooms to form products of the desired size, a high quality product is produced, devoid of defects, by a minimum number of rolling operations at a minimum cost.

In the appended claims the expression "blooms, slabs, billets and the like" is intended to include similar products such as plates and the like; the expression "arcuate blooms" is intended to include arcuate slabs; and the expression "arcuate bloom" is intended to include an arcuate slab.

We claim :

1. The method of making massive metal blooms, slabs, billets and the like which includes centrifugally molding an annular ring having non-parallel annular surfaces, severing the ring to form arcuate blooms having opposite arcuate surfaces and opposite non-parallel surfaces, and then straightening the arcuate blooms by passing the same through rolls engaging and applying pressure to the non-parallel surfaces.

2. The method of making massive metal blooms, slabs, billets and the like which includes centrifugally molding an annular ring having non-parallel annular surfaces, severing the ring to form arcuate blooms having a substantially trapezoidal shape in cross section with opposite non-parallel surfaces, and then straightening the arcuate blooms by passing the same through rolls engaging the non-parallel surfaces and compressing and displacing the metal between said surfaces.

3. The method of making massive metal blooms, slabs, billets and the like, which includes centrifugally molding an annular ring with an insulating material coating on its inner arcuate surface, said ring having non-parallel annular surfaces, severing the ring to form arcuate blooms having opposite arcuate surfaces and opposite non-parallel surfaces, the inner arcuate surface of the blooms having insulating material adhering thereto, and then rolling the non-parallel surfaces and compressing the arcuate blooms by pressure applied to said non-parallel surfaces to displace the metal at and adjacent to said last mentioned arcuate surface to loosen the material adhering thereto and to straighten the blooms.

4. The method of making massive metal blooms, slabs, billets and the like which includes centrifugally molding an annular ring having non-parallel annular surfaces, severing the ring to form arcuate blooms having opposite arcuate surfaces and opposite non-parallel surfaces, one of the arcuate surfaces being slightly concaved between the non-parallel surfaces, and then rolling the non-par-

allel surfaces and compressing the arcuate blooms between said non-parallel surfaces to extrude the metal at and adjacent to the said concaved arcuate surface to eliminate 5 the concavity and straighten the blooms.

5. The method of making massive metal blooms, slabs, billets and the like which includes centrifugally molding an annular ring having non-parallel annular surfaces, severing the ring to form arcuate blooms having opposite arcuate surfaces and opposite non-parallel surfaces, the blooms having sharp corners between the non-parallel surfaces and one of the arcuate surfaces, and then rolling 10 the non-parallel surfaces and compressing the arcuate blooms between said non-parallel surfaces to extrude the metal at and adjacent to the said sharp corners to eliminate the same and straighten the blooms.

20 6. The method of making massive blooms, slabs, billets and the like which includes centrifugally molding an annular ring having non-parallel annular surfaces, severing the ring to form arcuate blooms having opposite arcuate surfaces and opposite non-parallel surfaces, one of the arcuate surfaces being slightly concaved between the parallel surfaces and the corners between said arcuate surface and non-parallel surfaces being 25 sharp, and then rolling the non-parallel surfaces and compressing the arcuate blooms between said non-parallel surfaces to extrude the metal at and adjacent to the said concaved surface and sharp corners to eliminate 30 the concavity and sharp corners and straighten the blooms.

7. The method of making metal billets, plates and the like which includes centrifugally molding an annular ring having non-parallel annular surfaces, severing the ring to form an arcuate bloom having opposite arcuate surfaces and opposite non-parallel surfaces, then straightening the arcuate bloom by passing the same through rolls engaging and applying pressure to the non-parallel surfaces, and then rolling the straightened bloom by a plurality of passes to form billets, plates and the like.

8. The method of making massive blooms, 50 slabs, billets and the like which includes centrifugally molding an annular ring having non-parallel annular surfaces, severing the ring to form an arcuate bloom having opposite arcuate surfaces and opposite non-parallel surfaces, and then straightening the arcuate bloom by passing the same through rolls engaging and applying pressure to the non-parallel surfaces.

9. The method of making metal billets, 60 plates and the like which includes centrifugally molding an annular ring having non-parallel annular surfaces, severing the ring to form arcuate blooms having opposite arcuate surfaces and opposite non-parallel surfaces, then straightening the arcuate blooms

by passing the same through rolls engaging and applying pressure to the non-parallel surfaces, and then rolling the straightened blooms by a plurality of passes to form billets, plates and the like.

In testimony that we claim the above, we have hereunto subscribed our names:

HARRY M. NAUGLE.  
ARTHUR J. TOWNSEND.

70

75

80

85

90

95

100

105

110

115

120

125

130